

## UNITED STATES PATENT OFFICE.

TARIO KIKUTA, OF TOBATA CITY, FUKUOKA KEN, JAPAN, ASSIGNOR TO TOBATA IMONO KABUSHIKI KAISHA, OF TOBATA CITY, FUKUOKA KEN, JAPAN, A CORPORATION OF JAPAN.

METHOD OF MANUFACTURING BLACK-HEART MALLEABLE CAST IRON FROM WHITE CAST IRON.

No Drawing. Application filed September 29, 1926. Serial No. 138,575.

The present invention relates to improvements in a method of manufacturing black heart malleable cast iron, consisting in carrying out two stages of the graphitization which 5 takes place in manufacturing black heart malleable cast iron by annealing white cast iron and then immediately after completion of the second stage of graphitization immersing or quenching same in cold or boiling water or 10 exposing same in the open air. The object of the invention is to spare packing material which has hitherto been necessary for the annealing process and also to shorten the annealing time. Moreover, this invention does not 15 only produce castings of a uniform and superior quality, but also entirely prevents the black heart malleable cast iron from becoming brittle under heat treatment like hot galvanizing or sherardizing as when the ordinary 20 process of annealing is used and also, the superior quality of iron obtained by this invention will remain unaffected by a temperature below the freezing point of water.

To obtain black heart malleable cast iron 25 by annealing white cast iron, it is common to fill an annealing pot with white cast iron together with sand, a mixture of sand and iron oxides, air furnace slag, or ash; charge an annealing furnace with same; and heat it with 30 coal, coal gas, fuel oil or electric current at a temperature ranging from 850° C. to 920° C. for 70 to 100 hours. Then the pot is allowed to cool very slowly in the furnace. It being possible by this method to maintain a high temperature for a considerable length of time, it 35 is possible to complete the graphitization of free cementite, but since the eutectoid cementite produced at Ar<sub>1</sub> transformation point is graphitized only during the cooling period 40 of the furnace, the graphitization cannot be completed by the ordinary method when the quantities of carbon, silicon, and other elements contained in white cast iron are little, or the capacity of the furnace is small. As 45 regards the quality of black heart malleable cast iron produced, the perfect graphitization of this eutectoid cementite, as well as that of

the above free cementite, is of vital importance.

In an annealing according to my invention, 50 the packing material indispensable in the method hitherto known can be dispensed with. The proper temperature between 850° and 950° C. is kept up constantly for 15 to 60 hours in order to graphitize free cementite. 55 Then, the temperature is lowered to between 730° and 650° C., and after the temperature is maintained within this limit for 20 to 50 hours, the pot is taken out of the furnace and cooled in the open air. When a muffle furnace 60 is used, the product is either taken out and cooled in the open air or quenched in water. The temperatures and length of time to be thus constantly maintained should be selected 65 and properly kept within a given limit according to the chemical composition of the white cast iron.

Thus, according to my method it is possible 70 to prevent the imperfect graphitization of eutectoid cementite due to the shortage of carbon or silicon or the excess of the other elements contained in white cast iron such as manganese, sulphur and chromium which occurs in the method hitherto known. Besides, 75 it is possible to shorten the time required for heating and cooling the furnace, because I do not use the packing material indispensable in the old method which adds to the slowness of the cooling of a furnace due to its poor conductivity after the fire is extinguished, so that 80 the time of one cycle of annealing can be reduced considerably, for example, by nearly 3 or 4 days in a 10-ton furnace. Further, as 85 non-conductors of heat such as sand, iron oxide, slag, etc. are unnecessary, the operation is very much simplified, the annealing reduced, and the product obtained is of a superior and more uniform quality.

The black heat malleable cast iron manufactured by ordinary annealing methods becomes 90 very brittle as a rule, when subjected to a heat treatment such as hot galvanizing or sherardizing; that is to say, when heated at a temperature of 300° to 550° C. and then im-

mersed in cold or boiling water. However, the product made according to my invention retains its original quality permanently, even if subjected to a violent heat treatment. In fact, it may be heated to any temperature below  $Ar_1$  transformation point and then directly quenched in cold or boiling water or exposed to a temperature below the freezing point of the water.

10 To show a manner of carrying out the present invention in practice, I give below examples of annealing process with the annealing furnaces heated by pulverized coal (1) and electricity (2) respectively.

15

*Annealing furnaces used.*

(1) Is charged with about 10 tons of the product.

20 (2) Is charged with about 600 kilograms of the product.

*Method of charging.*

In (1), 66 malleable cast iron pots of cylindrical shape, 22 inches in diameter and 18 inches in height, filled with white cast iron, were used. They were put in the furnace three pots high and in twenty two stacks.

In (2), one mild steel pot of cylindrical shape, 600 millimeters in diameter and 850 millimeters in height, filled with white cast iron, was used.

*Method of annealing.*

35 In (1), the furnace was heated at  $900^{\circ} C.$  for 40 hours to complete the first stage of graphitization (mainly of free cementite). For the second stage of graphitization (chiefly of eutectoid cementite) a temperature of  $700^{\circ} C.$  was maintained for 40 hours. Soon after the fire was extinguished, the pots were taken out of the furnace and cooled in the open air as they are.

45 In (2), so as to carry out the first stage of graphitization the furnace was heated at  $920^{\circ} C.$  for 28 hours. Then, to complete the second stage of graphitization a temperature of  $710^{\circ} C.$  was maintained for 35 hours.

50 After that, the product was taken out of the furnace. Then a part of it was quenched in cold water and the rest exposed in the open air to effect rapid cooling.

*Result of annealing.*

55 As a means of test, first a part of the product was broken and the fracture examined. Then, tensile and bending tests were conducted with tensile and bending test pieces made of the same melt, which has been annealed in the same furnace with the products, and it was found out that it had been perfectly annealed, the fracture presenting a velvet-like grey color.

The following are the results of the tension and bending tests:—

| Treatment after the completion of the second stage of graphitization. | No. of test piece. | Tension test.                               |                                                     | Bend-<br>ing test<br>(inner<br>radius<br>35 mm.) | 70 |
|-----------------------------------------------------------------------|--------------------|---------------------------------------------|-----------------------------------------------------|--------------------------------------------------|----|
|                                                                       |                    | Tensile strength<br>(kg./mm. <sup>2</sup> ) | Elongation<br>in %<br>(gauge<br>length =<br>50 mm.) |                                                  |    |
| Air cooled products in the annealing pot.                             | 995 A              | 36.50                                       | 16.0                                                | 180                                              | 75 |
|                                                                       | 995 B              | 37.60                                       | 16.5                                                | 180                                              |    |
|                                                                       | 995 C              | 36.75                                       | 15.5                                                | 180                                              |    |
| Air cooled products taken out of the pot.                             | 996 A              | 37.50                                       | 15.5                                                | 180                                              |    |
|                                                                       | 996 B              | 36.90                                       | 15.5                                                | 180                                              |    |
|                                                                       | 996 C              | 38.00                                       | 16.5                                                | 180                                              |    |
| Quenched in the water, products taken out of the pot.                 | 997 A              | 37.70                                       | 16.5                                                | 180                                              | 80 |
|                                                                       | 997 B              | 39.85                                       | 15.5                                                | 180                                              |    |
|                                                                       | 997 C              | 38.18                                       | 16.0                                                | 180                                              |    |

The tension test pieces used in the above test were  $\frac{5}{8}$  inch in diameter, and the bending test pieces had a section of  $\frac{3}{8}$  inch in thickness and  $\frac{5}{8}$  inch in breadth.

Next, the black heart malleable cast iron manufactured by the annealing method of my invention and the malleable cast iron manufactured by an ordinary process were subjected to a heat treatment similar to those required for hot galvanizing or sherardizing; that is to say, heated at a temperature of  $450^{\circ} C.$  for 20 minutes; and then immersed in the cold water. After being thoroughly cooled, they were subjected to an impact test, and the following results were obtained (the same result was obtained with boiling water instead of cold water, and therefore, that result is omitted):—

| Black heart malleable cast iron manufactured by annealing according to the present invention. | Black heart malleable cast iron manufactured by annealing according to the present invention. |                            |                                                                                             |                            |                                                                                      |                            |
|-----------------------------------------------------------------------------------------------|-----------------------------------------------------------------------------------------------|----------------------------|---------------------------------------------------------------------------------------------|----------------------------|--------------------------------------------------------------------------------------|----------------------------|
|                                                                                               | Cooled in the air in a pot after the completion of the second stage of graphitization.        |                            | Cooled in the air outside a pot after the completion of the second stage of graphitization. |                            | Cooled in the cold water after the completion of the second stage of graphitization. |                            |
|                                                                                               | Before the heat treatment.                                                                    | After the heat treatment.  | Before the heat treatment.                                                                  | After the heat treatment.  | Before the heat treatment.                                                           | After the heat treatment.  |
| Before the heat treatment.                                                                    | After the heat treatment.                                                                     | Before the heat treatment. | After the heat treatment.                                                                   | Before the heat treatment. | After the heat treatment.                                                            | Before the heat treatment. |
| 1.31                                                                                          | 0.11                                                                                          | 1.51                       | 1.18                                                                                        | 1.57                       | 1.57                                                                                 | 1.50                       |
| 1.15                                                                                          | 0.15                                                                                          | 1.57                       | 1.31                                                                                        | 1.57                       | 1.47                                                                                 | 1.39                       |
| 1.31                                                                                          | 0.11                                                                                          | 1.51                       | 1.12                                                                                        | 1.57                       | 1.70                                                                                 | 1.41                       |

For the above impact test, a Charpy impact testing machine and the standard notched bars were used and the meter-kilogram system was adopted as units.

From the above it will be seen that the black heart malleable cast iron manufactured according to the methods of annealing of this invention undergoes no change in the quality under a heat treatment such as is used for hot galvanizing or sherardizing.

The above is merely one example of the annealing done according to this invention,

and although the temperature and the time of heating should receive due consideration according to the size of a furnace and the method of heating it, etc., the essential point 5 is to cool rapidly the product after carrying out the complete graphitization of the combined carbon contained in the white cast iron in two stages.

I claim—

- 10 1. A method of manufacturing black heart malleable cast iron from white cast iron without using packing material which comprises first maintaining the white cast iron at a temperature between 850° and 950° C. for 15 to 15 60 hours, then cooling the iron to a temperature between 730° and 650° C., and then

maintaining the iron at the latter temperature for 20 to 50 hours.

2. A method of manufacturing black heart malleable cast iron from white cast iron without using packing material which comprises 20 first maintaining the white cast iron at a temperature between 850° and 950° C. for 15 to 60 hours, then cooling the iron to a temperature between 730° and 650° C., then 25 maintaining the iron at the latter temperature for 20 to 50 hours, and then removing the iron from the furnace and cooling it rapidly.

In testimony whereof I have affixed my 30 signature.

TARIO KIKUTA.